

11

3,685,976

**MOTOR FUEL CONTAINING DIIMINE ADDITIVES**  
Jan H. Vis, Hengelo, Netherlands, and Wallace R. Loder,  
Jr., North Olmsted, Ohio, assignors to The Standard  
Oil Company, Cleveland, Ohio  
No Drawing. Filed May 24, 1971. Ser. No. 146,541

NO Drawing. Filed May 24, 1971, Ser. No. 146,841  
Int. Cl. C10l 1/22

U.S. Cl. 44—69

## 5 Claims

## **ABSTRACT OF THE DISCLOSURE**

Certain diimine compounds, characterized as the 1,3-diimino-2-hydroxypropanes, are effective for improving the antiknock performance and ignitability of motor fuels employed in high compression, spark-ignition-type engines.

This invention relates to an improved liquid motor fuel additive composition and more particularly to a motor fuel composition for use in high compression, spark-ignition engines containing minor amounts of diimine compounds. The motor fuel additives contemplated to be within the scope of this invention may be characterized as the 1,3-diimino-2-hydroxypropanes corresponding to the following general formula:



wherein R and R<sub>1</sub> may be the same or different and wherein R and R<sub>1</sub> may be an alkyl or a substituted alkyl group containing from about 3 to 10 carbon atoms, a cycloalkyl or a substituted cycloalkyl group containing from about 4 to 10 carbon atoms, or an aromatic or a substituted aromatic hydrocarbon group, containing from about 6 to 10 carbon atoms. The substituent groups on the foregoing R and R<sub>1</sub> radicals may be alkyl, hydroxy, methoxy, carbonyl, carboxyl, halogen, nitro or amine groups. The R<sub>2</sub>, R<sub>3</sub>, R<sub>4</sub> and R<sub>5</sub> radicals may be hydrogens or methyl groups.

It is well-known that during the operation of an initially clean internal combustion engine, deposits form progressively and accumulate on the surfaces within the combustion zone, and as the operation continues, the amount of the deposits reaches a level after which there is no appreciable further increase in the amount of the deposits. The engine is then regarded as having reached deposit equilibrium, and old deposits flake off as fast as new deposits form.

The deposit problem is aggravated when tetraethyl lead is contained in the fuel because the deposits are then no longer essentially carbonaceous, but comprise appreciable quantities of lead and lead compounds generally mixed with the carbonaceous material. The fact that this deposit is partially metallic in character is thought to give it a catalytic activity which modifies the action of the deposit in affecting engine operation.

These deposits have a number of adverse effects upon engine operation. One adverse effect of the deposits is manifested by an increase in the octane requirement of the engine. This requirement for a fuel of higher octane number as the engine becomes progressively dirtier, persists until the deposits reach equilibrium, and is known as octane requirement increase (ORI).

In addition to the adverse effects of combustion chamber deposits, approximately one-third of all cars on the

2

highways suffer from subnormal ignition. Some of these ignition difficulties arise from weak batteries in starting, worn points, oil and water-soaked electrical wiring known as harness, frayed or broken harness, weak coils, etc. All of these deficiencies tend to diminish the voltage delivered to the spark plugs.

The spark plugs themselves may contribute to ignition difficulties as well. With use, the electrodes erode, increasing the breakdown voltage of the gap. The lead from the binding post to the center electrode may break, requiring additional voltage to leap across that break as well as across the gap. The ceramic surfaces of the spark plug become fouled with deposits which act as short circuits and drain the voltage from the electrodes.

The resulting situation is that both use and abuse steadily raise the voltage required to jump the spark across the proper gap, while at the same time the voltage available at the gap steadily declines as the car ages. At some point in this process of deterioration, less voltage will be delivered to the electrodes than is required, and the spark will not jump the gap. The result of this deteriorating situation is difficult starting, misfiring or late firing, loss of power, especially during acceleration or hill climbing, and increased air pollution.

It is therefore an object of this invention to provide a motor fuel formulation that will alleviate the above problems that are common to the majority of spark-ignition-type automotive vehicles that are presently on the road. The additives of this invention are believed to promote ionization of the fuel thus improving conductivity of the gases contained in the spark plug gap, and they are also combustion chamber deposit modifiers. When added to motor fuels in minor amounts, the additives of this invention are effective in lowering the octane requirement, in minimizing the octane requirement increase and generally improving the antiknock performance of a fuel in a spark-ignition-type engine. The diimine additives of this invention are believed to be metal complexing agents, and it is postulated that when they are added to motor fuels containing organolead antiknock agents they interact with some of the lead during the combustion process and further improve the antiknock performance of the lead, thereby also functioning as lead appreciators.

U.S. Patent No. 3,248,410 issued Apr. 26, 1966 discloses the preparation of a monomeric polymerizable heavy metal chelate complex of the diimine structure shown herein above, and its use in modifying the burning rate properties of solid polymeric propellant binders. However, the use of these diimine compounds for improving octane performance and ignitability of motor fuels according to the present invention has heretofore not been proposed.

In accordance with this invention, diimines of the above designation may be added advantageously to leaded or unleaded motor fuels in concentrations ranging from about 100 parts to 1000 parts per million based on the fuel. Although improved performance may also be obtained at higher concentrations, the solubility limits in the fuel for most diimines is exceeded above this concentration level. Examples of some diimine compounds that fall within the scope of this invention are the following:



### N,N'-disalicylidene-2-hydroxy-1,3-propyldiimine

3



N,N'-dibenzylidene-2-hydroxy-1,3-propyldiimine



N,N'-di(2-pentylidene-4-one)-2-hydroxy-1,3-propyldiimine



N,N'-dihexahydrobenzylidene-2-hydroxy-1,3-propyldiimine



N,N'-disalicylidene-2-hydroxy-1,3-dimethyl-1,3-propyldiimine

When an organolead antiknock agent such as tetraethyl lead is present in the fuel, the fuel may also contain a lead scavenging agent such as a volatile alkyl halide or a mixture of volatile alkyl halides such as ethylene dichloride and/or ethylene dibromide as is well-known in the art. These halides are usually present as 1 theory of ethylene dichloride and  $\frac{1}{2}$  theory of ethylene dibromide (the so-called "motor mix") or 1 theory of ethylene dibromide (the so-called "aviation mix"). By "theory" is meant the stoichiometric amount of the ethylene dihalide for combination with all of the lead as lead halide.

The base gasoline stock useful as fuel in this invention can comprise a mixture of hydrocarbons boiling in the gasoline range and can be either a straight-run gasoline or a gasoline obtained from a conventional cracking process, or mixtures thereof. The base gasoline may also contain components obtained from various other refinery processes, such as alkylation, isomerization, hydrogenation, polymerization, catalytic reforming, or combinations of two or more of such processes.

It is intended that the motor fuel of this invention may also include other known additives for commercial fuels, such as detergents, oxidation inhibitors, gum inhibitors, deicers, dyes, solvent oils and the like.

To determine the effect of diimines on the octane rating of leaded and unleaded motor fuels, blended fuels were

4

evaluated in the standard ASTM (research) and ASTM (motor) octane test procedures. In these tests additive compositions, additive and tetraethyl lead concentrations were varied and the results were compared with tertiary butyl acetate at its most effective concentration. The effect of the additives on the octane rating of motor fuels is demonstrated by the examples given in Tables II, III and IV.

The physical and chemical properties of the base fuel employed in the octane test program were as follows:

TABLE I

|    |                          | ° F. |
|----|--------------------------|------|
|    | Distillation:            |      |
| 15 | Initial B.P.             | 94   |
|    | 10%                      | 133  |
|    | 50%                      | 219  |
|    | 90%                      | 333  |
|    | E.P.                     | 394  |
| 20 | Percent recovered        | 98   |
|    | Percent residue          | 1    |
|    | Percent loss             | 1    |
|    | Gravity, °API            | 60.2 |
|    | RVP                      | 8.1  |
| 25 | Octane ASTM research     | 93.1 |
|    | Octane ASTM motor        | 83.6 |
|    | TEL, cc./gal.            | 0    |
|    | Composition:             |      |
| 30 | Lt. isocrackate          | 24   |
|    | Lt. catalytic distillate | 19   |
|    | Total catalytic reformat | 35   |
|    | Alkylate                 | 18   |
|    | Natural gasoline         | 4    |
| 35 |                          |      |

TABLE II

| 40 | Example No. | Additive                       | Conc., moles/gal. | Tetraethyl, lead, cc./gal. | Increase in octane No. over base fuel without additive |
|----|-------------|--------------------------------|-------------------|----------------------------|--------------------------------------------------------|
|    |             |                                |                   |                            | ASTM research octane rating                            |
| 1  |             | N,N'-disal. hyd. <sup>1</sup>  | 0.0696            | 0                          | 2.6                                                    |
| 2  |             | N,N'-dipent. hyd. <sup>2</sup> | 0.0174            | 0                          | 1.3                                                    |
| 3  |             | Tert. butyl acetate            | 0.0696            | 0                          | 0.9                                                    |
| 4  |             | N,N'-disal. hyd.               | 0.0696            | 1                          | 4.1                                                    |
| 5  |             | N,N'-dipent. hyd.              | 0.0174            | 1                          | 3.7                                                    |
| 6  |             | Tert. butyl acetate            | 0.0696            | 1                          | 3.4                                                    |
| 7  |             | N,N'-disal. hyd.               | 0.0696            | 3                          | 1.3                                                    |
| 8  |             | N,N'-dipent. hyd.              | 0.0696            | 3                          | 1.1                                                    |
| 9  |             | Tert. butyl acetate            | 0.0696            | 3                          | 1.8                                                    |
| 50 |             |                                |                   |                            | ASTM motor octane rating                               |
| 10 |             | N,N'-disal. hyd.               | 0.0696            | 0                          | 1.0                                                    |
| 11 |             | N,N'-dipent. hyd.              | 0.0174            | 0                          | -1.4                                                   |
| 12 |             | Tert. butyl acetate            | 0.0696            | 0                          | -0.2                                                   |
| 13 |             | N,N'-disal. hyd.               | 0.0696            | 1                          | 1.0                                                    |
| 14 |             | N,N'-dipent. hyd.              | 0.0174            | 1                          | 0.4                                                    |
| 15 |             | Tert. butyl acetate            | 0.0696            | 1                          | 0.1                                                    |
| 16 |             | N,N'-disal. hyd.               | 0.0696            | 3                          | 1.3                                                    |
| 17 |             | Tert. butyl acetate            | 0.0696            | 3                          | 1.9                                                    |

<sup>1</sup> N,N'-disal. hyd.=N,N'-disalicylidene-2-hydroxy-1,3-propyldiimine.

<sup>2</sup> N,N'-dipent. hyd.=N,N'-di(2-pentylidene-4-one)-2-hydroxy-1,3-propyldiimine.

Examples 1 to 17 shown in Table II indicate that at zero concentration of tetraethyl lead the diimine compounds show antiknock behavior by themselves, and a greater octane response is indicated for these additives than for an equivalent concentration of tertiary butyl acetate. The increase in octane response resulting from the diimine additive is not as great with increasing concentrations of tetraethyl lead, however, the increase in octane ratings of leaded fuel attributable to the diimine additive is still appreciable.

The effect of diimine compounds on the control of octane requirement increase of a fuel was measured in a 100-hour single cylinder test. The tests were conducted in a Waukesha CFR-48 octane engine coupled to a variable speed dynamometer so as to provide cycling

capability. The test fuel employed in these tests was the same as that shown in Table I. The test cycle conditions were as follows:

## CYCLING SCHEDULE

|                              |             |                |
|------------------------------|-------------|----------------|
| Cycle duration, seconds..... | 55.....     | 145.....       |
| Cycle speed, r.p.m.....      | 600.....    | 900.....       |
| Throttle setting.....        | Idle.....   | Wide open..... |
| Air/fuel ratio.....          | 11.5:1..... | 13:1.....      |

## Test conditions:

Length of run—100 hours  
Ignition timing—6° BTDC  
Compression ratio, nominal—9:00:1  
Coolant temperature—220° F.  
Oil temperature—150° F.  
Inlet air temperature—100° F.  
Spark plug gap—0.020"

Octane requirements were determined at the start of the experiment and once each day thereafter. The method consisted of introducing known octane number primary reference fuels into the carburetor at an air/fuel ratio of 13:1, and advancing the spark to produce trace audible knock at wide open throttle. Three reference fuels were used having octane numbers such that the spark advance of 6° BTDC could be bracketed. The octane requirement at 6° BTDC was then determined by interpolation from a curve relating octane requirement to spark advance.

engine has a lower octane requirement after the additive fuel has been run than before. This effect is demonstrated by Examples 24 to 34 given in Table IV. It is also seen that the higher the additive concentration, the stronger the "aftereffect," both in length and intensity.

To determine the effect of the diimine additives on the ignitability of motor fuel, acceleration tests were carried out in a 302 cubic inch 1970 Ford V-8 engine. The test employed measured the ability of a gasoline to deliver power under a variety of conditions ranging from those producing severe misfiring to those producing no misfiring. Critical performance occurred during acceleration at wide open throttle. The means for inducing misfire consisted of reducing the voltage available at the primary winding of the spark coil to a substandard level. Under these conditions, the power output of the engine was reduced below that level normally observed at full ignition voltage. The increase in power output of the additive fuel compared with the base fuel in terms of horsepower was employed as a measure of the ability of the additive to improve the ignitability of the fuel.

In the tests carried out in the instant invention, the engine was coupled to an Eaton Dynamatic "Universal" dynamometer. The engine was equipped with a finely adjustable ignition voltage supply and a digital voltmeter. In conducting these tests, the engine power output was adjusted to a target level using the base fuel, and tests were then run between power levels of 65 percent and

TABLE IV  
[Additive: N,N'-disalicylidene-2-hydroxy-1,3-propyldiimine]

| Example No.                          | Tetraethyl lead, cc./gal. | Conc. of addit., moles/gal. | Duration of "After-effect," min. | Minutes  |          |          |          |
|--------------------------------------|---------------------------|-----------------------------|----------------------------------|----------|----------|----------|----------|
|                                      |                           |                             |                                  | 4        | 8        | 16       | 32       |
| <b>ASTM research test conditions</b> |                           |                             |                                  |          |          |          |          |
| 24.....                              | 0.....                    | 0.0696.....                 | 35.....                          | 1.2..... | 1.0..... | 1.0..... | 0.2..... |
| 25.....                              | 0.....                    | 0.0343.....                 | 89.....                          | 0.3..... | 0.2..... | .....    | .....    |
| 26.....                              | 1.....                    | 0.0696.....                 | >70.....                         | 1.6..... | 1.6..... | 1.6..... | .....    |
| 27.....                              | 1.....                    | 0.0348.....                 | 13.....                          | 0.6..... | 0.6..... | .....    | .....    |
| 28.....                              | 3.....                    | 0.0696.....                 | >30.....                         | 1.6..... | 1.6..... | 1.5..... | 1.8..... |
| <b>ASTM motor test conditions</b>    |                           |                             |                                  |          |          |          |          |
| 29.....                              | 0.....                    | 0.1392.....                 | 28.....                          | 2.0..... | 4.0..... | 1.3..... | .....    |
| 30.....                              | 0.....                    | 0.0696.....                 | 60.....                          | 1.0..... | 3.0..... | 4.0..... | 4.0..... |
| 31.....                              | 0.....                    | 0.0174.....                 | 68.....                          | 0.4..... | 0.5..... | 0.6..... | 0.7..... |
| 32.....                              | 1.....                    | 0.0696.....                 | >18.....                         | 4.0..... | 4.0..... | 4.0..... | .....    |
| 33.....                              | 1.....                    | 0.0348.....                 | 30.....                          | 0.9..... | 0.9..... | 0.9..... | .....    |
| 34.....                              | 3.....                    | 0.0696.....                 | >60.....                         | 2.5..... | 2.0..... | 1.7..... | .....    |

The results of measurements of octane requirement increase (ORI) of the fuel are summarized in Table III. The data show that ORI of the engine is reduced considerably with fuels containing the diimine additives.

Another effect that is characteristic of fuels containing the diimine additive of this invention is "aftereffect." Under normal circumstances, the reference fuel octane response is the same before and after running the additive fuel in the engine. The time required for the reference fuel to return to previous octane level after running the additive fuel is approximately 2 to 5 minutes. This time is considerably longer for fuels containing the diimine additives so that the reference fuel has a higher octane number after the additive fuel has been run in the engine than before. Expressing this effect in another way, the

TABLE III.—100 HOUR TEST

| Example No. | Additive conc., p.p.m. | Tetraethyl lead, g./gal. | Octane requirement increase (ORI) | Difference from base (ORI) |
|-------------|------------------------|--------------------------|-----------------------------------|----------------------------|
| 18.....     | Base fuel.....         | 0.....                   | 9.0.....                          | .....                      |
| 19.....     | do.....                | 0.5.....                 | 9.5.....                          | .....                      |
| 20.....     | 200 <sup>1</sup> ..... | 0.....                   | 4.5.....                          | -5.5.....                  |
| 21.....     | 200 <sup>1</sup> ..... | 0.5.....                 | 4.5.....                          | -3.0.....                  |
| 22.....     | 200 <sup>2</sup> ..... | 0.....                   | 6.0.....                          | -4.0.....                  |
| 23.....     | 200 <sup>2</sup> ..... | 0.5.....                 | 8.0.....                          | -1.5.....                  |

<sup>1</sup> N,N'-disalicylidene-2-hydroxy-1,3-propyldiimine.<sup>2</sup> N,N'-dibenzylidene-2-hydroxy-1,3-propyldiimine.

50 100 percent of full power, as determined with the base fuel. The additive-containing fuels were evaluated in a series of tests with base fuels interspersed as reference points. The engine test cycle involved acceleration and idling under the following conditions:

| Phase  | "N," r.p.m.            | "T," load      | H.P.          | Time, seconds |
|--------|------------------------|----------------|---------------|---------------|
| 1..... | Idle @ 1200.....       | 12 lb. ft..... | 4.5.....      | 60.....       |
| 2..... | Accel. to x r.p.m..... | Variable.....  | Variable..... | 6.....        |
| 3..... | Cruise @ 2000.....     | 72 lb. ft..... | 48.....       | 60.....       |

60 The cycle was run under the following conditions:

Water jacket outlet temperature, ° F.—165±5

Oil sump temperature—Equilibrium

Carburetor adjustments—Factory specification

Inlet air, ° F.—80

During the acceleration part of the cycle, the engine performance increased with respect to both speed and torque and performance of the fuel was calculated by means of the following formula employing the speed and torque readings at the end of the 6 second acceleration period:

$$\text{Terminal H.P.} = \frac{\text{Torque} \times \text{r.p.m.}}{\text{Dynamometer constant}}$$

Data produced from the above tests were fed into a computer to obtain a regression equation based on a full quadratic model.

The base fuel used in the acceleration tests had the specifications shown in Table V.

TABLE V

| Distillation:            | ° F.           |
|--------------------------|----------------|
| IBP                      | 88             |
| 10%                      | 125            |
| 50%                      | 214            |
| 90%                      | 331            |
| EP                       | 396            |
| Percent recovered        | 98             |
| Percent residue          | 1.0            |
| Percent loss             | 1.0            |
| Gravity, ° API           | 61.3           |
| RVP                      | 9.7            |
| Octane ASTM (research)   | 100.4          |
| Octane ASTM (motor)      | 92.7           |
| TEL, cc./gal.            | 2.98           |
| Composition:             | Volume percent |
| Lt. isocrackate          | 22             |
| Lt. catalytic distillate | 18             |
| Catalytic reformate      | 33             |
| Alkylate                 | 20             |
| Natural gas              | 4              |
| N-butane                 | 3              |
| SEB-78                   | 0.25           |

The effect of the various imine compounds on power delivery of the fuel is shown by the examples given in Table VI.

TABLE VI

| Example No.                                                       | p.p.m. additive | Fractional power level | Horsepower |
|-------------------------------------------------------------------|-----------------|------------------------|------------|
| Additive: N,N'-disalicylidene-2-hydroxy-1,3-propyldiimine         |                 |                        |            |
| 35-----                                                           | 50              | .89                    | -5.54      |
|                                                                   | 100             | .89                    | -6.88      |
|                                                                   | 200             | .85                    | -1.01      |
|                                                                   | 300             | .80                    | +6.39      |
|                                                                   | 400             | .87                    | +8.43      |
|                                                                   | 554             | .80                    | +10.80     |
|                                                                   | 600             | .88                    | +5.33      |
|                                                                   | 180             | .95                    | +0.70      |
|                                                                   | 100             | .95                    | +0.54      |
|                                                                   | 200             | .95                    | +0.35      |
| Additive: N,N'-dihexahydrobenzylidene-2-hydroxy-1,3-propyldiimine |                 |                        |            |
| 36-----                                                           | 183             | .95                    | +1.72      |
|                                                                   | 183             | 1.00                   | +0.26      |
| Additive: N,N'-dibenzylidene-2-hydroxy-1,3-propyldiimine          |                 |                        |            |
| 37-----                                                           | 200             | 1.00                   | +0.61      |

We claim:

1. A motor fuel composition for internal combustion engines containing from about 100 parts to 1000 parts per million based on the motor fuel of a diimine compound having the formula:



wherein R and R<sub>1</sub> may be the same or different and wherein R and R<sub>1</sub> may be selected from the group consisting of an alkyl or a substituted alkyl group containing from about 3 to 10 carbon atoms, a cycloalkyl or a substituted cycloalkyl group containing from about 4 to 10 carbon atoms, and an aromatic or a substituted aromatic group containing from about 6 to 10 carbon atoms, and wherein the substituting groups on said foregoing R and R<sub>1</sub> radicals may be alkyl, hydroxy, methoxy, carbonyl, carboxyl, halogen, nitro or amine groups, and R<sub>2</sub>, R<sub>3</sub>, R<sub>4</sub> and R<sub>5</sub> may be hydrogens or methyl groups.

2. The motor fuel composition of claim 1 wherein the fuel contains up to 6 cc. of tetraalkyl lead per gallon and a halide scavenging agent.

3. The motor fuel composition of claim 1 wherein the diimine compound is a member selected from the group consisting of N,N'-disalicylidene-2-hydroxy-1,3-propyldiimine, N,N'-dibenzylidene-2-hydroxy-1,3-propyldiimine, N,N'-di(2-pentylidene-4-one)-2-hydroxy-1,3-propyldiimine and N,N'-dihexahydrobenzylidene-2-hydroxy-1,3-propyldiimine.

4. The motor fuel composition of claim 3 wherein the diimine compound is N,N'-disalicylidene-2-hydroxy-1,3-propyldiimine.

5. The motor fuel composition of claim 3 wherein the diimine compound is N,N'-dibenzylidene-2-hydroxy-1,3-propyldiimine.

#### References Cited

##### UNITED STATES PATENTS

- |         |           |         |            |           |       |
|---------|-----------|---------|------------|-----------|-------|
| 45----- | 2,533,205 | 12/1950 | Chenicek   | -----     | 44-73 |
|         | 2,626,208 | 1/1953  | Brown      | -----     | 44-73 |
|         | 3,034,876 | 5/1962  | Gee et al. | -----     | 44-73 |
|         | 3,248,410 | 4/1966  | Berenbaum  | 260-439 R |       |

50 PATRICK P. GARVIN, Primary Examiner

Y. H. SMITH, Assistant Examiner

U.S. Cl. X.R.

44-73